

# United States Patent Office

2,909,514

Patented Oct. 20, 1959

1

2,909,514

## MANUFACTURE OF ROSIN AND ROSIN SIZE OF DECREASED LATENT FOAMING TENDENCY

Lucius H. Wilson and William C. Hopkins, Valdosta, Ga., and Stanley F. Stafiej, Stamford, Conn., assignors to American Cyanamid Company, New York, N.Y., a corporation of Maine

No Drawing. Application March 7, 1957  
Serial No. 644,450

8 Claims. (Cl. 260—97)

The present invention relates to a method for treating rosins containing alcoholic foam-producing components. More particularly, the invention relates to the heating of such rosins with oxidic boron material to decrease the foaming tendency caused by such components when such rosins are converted to rosin size and used in the manufacture of paper. The invention includes liquid rosin size prepared from the thus-treated rosins.

The manufacture of sized paper on a commercial scale is generally performed by beating wood or other cellulosic fibers in aqueous suspension until the fibers have become well hydrated, sizing the fibers by adding rosin size and alum to the fibrous suspension, and discharging the suspension upon a moving wire of a Fourdrinier machine to form a web which becomes paper when subsequently dried and calendered. In the process the aqueous fibrous suspension is unavoidably subjected to continuous vigorous agitation and aeration throughout its journey to the wire. It consequently normally tends to develop foam.

The success of the paper-making process depends upon the laying down of suspended fibers in uniform fashion on the Fourdrinier wire so that the web is continuous and homogeneous. Satisfactory paper is not formed when the fibrous suspension contains foam as it is delivered to the wire as the foam causes the fibers to form into bunches, so that it is laid in discontinuous fashion. In such event the wet web and the resulting paper may contain weak spots or even holes. Paper having pin holes or larger discontinuities is not commercially acceptable.

Natural rosin (particularly gum rosin and wood rosin) has pronounced latent tendency to foam (i.e., tendency to foam when converted into dilute aqueous sodium rosinate solution and agitated).

We have investigated such rosin in the laboratory to determine the cause of its tendency to foam and our evidence is that this foaming is due to the presence in the rosin of small amounts of organic alcohols. The present invention is principally based upon our discovery that these alcohols may be rapidly, cheaply, and if desired, substantially completely inactivated by the chemical action of certain compounds of boron thereon.

We have found that the latent foaming tendency of such rosin can be decreased by heating the rosin in molten form with an oxidic compound of boron at a temperature between about 150° C. and 250° C. If desired, the rosin may be heated with sufficient of the boron compound and for a sufficient time to effect inactivation of substantially all of the alcoholic foam-forming materials present, so that the latent foaming tendency of the rosin is substantially completely negated. Thereafter, the rosin may be converted to liquid rosin size in normal manner by saponification with aqueous alkali metal alkali solution.

The above described process has the following principal advantages:

(1) It does not require the rosin to be heated to a

2

temperature where significant darkening, decarboxylation or other degradation occurs. In certain instances the acid number of the rosin has been observed to increase during the treatment, perhaps as a result of volatilization of the foam-producing components.

(2) Small amounts of preferred boron compounds are effective, but excess amounts thereof are tolerated without harm. The temperature range and reaction time being broad, the invention does not depend on the observance of narrowly critical limitations.

(3) The treatment does not introduce any limitation into the utility of the rosin. The treated rosin may thus be fortified according to procedures heretofore known (e.g., by reaction with saligenin, maleic anhydride, para-formaldehyde, etc.) and may be converted into liquid and dry size in the same manner as ordinary rosin, i.e., rosin which has not been so treated.

(4) The procedure does not involve the addition of solvent material to the rosin, filtration of the rosin, or distillation of the rosin. It thus does not require the rosin manufacturer or rosin size manufacturer to vary established procedures.

More in detail, according to one preferred embodiment of the invention, the rosin to be treated is first brought to fluid molten condition at about 175° C.—200° C. in a closed or open vessel equipped with a stirrer. The alcohol-reactive oxidic boron compound is then slowly added with vigorous stirring so as to effect a controlled uniform reaction, the temperature being maintained within the range stated. The rosin is maintained at reaction temperature until the reaction is complete and any volatile material formed has substantially completely escaped.

The amount of boron compound which is added in any instance chiefly depends upon the temperature and the duration of the heating, the extent to which it is desired to decrease the latent foaming capacity of the rosin, and the effectiveness of the particular boron compound as agent for the purpose. In practice, we prefer to heat the rosin with sufficient of the boron compound and for a sufficient time to inactivate between about  $\frac{1}{3}$  and  $\frac{3}{4}$  of the foam-producing components of the rosin. In this range, consumption of the boron compound is minimized while the foaming index of the rosin is substantially improved.

The invention does not require any temperature higher than 250° C. This temperature is sufficiently high to convert the foam-producing agents to inactive form, yet is sufficiently low that the rosin is not decarboxylated or otherwise harmed. Rosin is sensitive to oxidation, and it is accordingly advantageous to blanket the surface of the rosin during the treatment with nitrogen or other inert gas. We prefer to use a temperature in excess of about 150° C. as below this temperature the reaction rate is uneconomically slow.

The reaction proceeds satisfactorily at atmospheric pressure but where volatile organic products form, the reaction is often accelerated by diminished pressure. Very low pressures, however, cause rosin to boil and distill in the range 225° C.—250° C. If such low pressures are employed, the temperature of the rosin should be decreased so as to maintain the rosin below its boiling point, as according to the invention the rosin is not distilled.

The boron compounds which may be used in the process of the present invention include the boron acids, the boron oxides and the higher organic substituted boron acids and oxides. Thus there may be employed monosodium orthoborate, monosodium pyroborate, trioctadecyl borate and trioleyl borate, tributyl borates, and phenylboronic acid. We prefer to employ boric acid and

boric anhydride as these compounds are easily handled, readily available, and more effective per unit weight than most of the other compounds. It will be understood that the boron compound may undergo thermal decomposition before reacting, and that treatment of the rosin with the decomposition product is within the scope of the invention.

The invention does not depend upon the addition of any particular amount of boron compound, the particular heating temperature employed, or the duration of the heating period. As stated, we prefer to add sufficient of the boron compound and to heat for a sufficiently long time at a sufficiently high temperature so as to inactivate between one-third and about three-quarters of the alcoholic foam-producing components present.

The optimum amount of the boron compound to be added in any one instance may be readily determined by making a series of laboratory trials as illustrated in the examples below and determining the foaming index of the rosin product by the standard laboratory methods shown in U.S. Patent No. 2,471,714. When rated according to this test, gum rosin generally has a foaming index

hour thereafter. The foaming index of the rosin was then determined, and in certain instances the acid number as well.

The foaming index of the rosin was determined by the following procedure as described in U.S. Patent No. 2,471,714:

The rosin was converted to a 70% solids, 12% free acid liquid size by reaction with the calculated amount of aqueous sodium hydroxide solution. The size was then diluted to 5% solids with water. To 20 cc. of this solution there was added 5 cc. of a 10% solution of papermakers alum,  $Al_2(SO_4)_3 \cdot 14H_2O$ . The mixture was then poured into 180 cc. of water and agitated for 1 minute in a high-speed laboratory Hamilton-Beach mixer. The dispersion was then poured into a 500-cc. graduate and the volume of foam measured. The foaming index, expressed in percent, is the ratio of the volume of foam to the volume of the liquid present before the test and is found according to the following formula:

$$\frac{\text{Total volume (liquid+foam)} - 205}{205 \text{ (volume of liquid)}}$$

| Run No. | Rosin | Heating    |            | Boron Cpd.           |         | Product Acid No. | Foam Index |
|---------|-------|------------|------------|----------------------|---------|------------------|------------|
|         |       | Temp., °C. | Time, Hrs. | Name                 | Percent |                  |            |
| Control | Gum   | 155        | 1          | None                 |         | 171              | 30         |
| 1       | do    | 155        | 1          | $B(OH)_3$            | 1       | 177              | 27         |
| 2       | do    | 155        | 1          | $B(OH)_3$            | 2       | 173              | 25         |
| 3       | do    | 155        | 1          | $B(OH)_3$            | 5       | 177              | 22         |
| 4       | do    | 165        | 1          | $B(OH)_3$            | 1       |                  | 27         |
| 5       | do    | 165        | 1          | $B(OH)_3$            | 2       | 176              | 17         |
| 6       | do    | 165        | 1          | $B(OH)_3$            | 5       |                  | 10         |
| 7       | do    | 175        | 1          | $B(OH)_3$            | 1       |                  | 22         |
| 8       | do    | 175        | 1          | $B(OH)_3$            | 2       |                  | 15         |
| 9       | do    | 175        | 1          | $B(OH)_3$            | 5       |                  | 5          |
| 10      | do    | 185        | 1          | $B(OH)_3$            | 1       |                  | 15         |
| 11      | do    | 185        | 1          | $B(OH)_3$            | 2       |                  | 10         |
| 12      | do    | 185        | 1          | $B(OH)_3$            | 5       |                  | 0          |
| 13      | do    | 165        | 1          | $B(OC_2H_5)_2(OH)_2$ | 3       |                  | 18         |
| 14      | do    | 175        | 1          | $B_2O_3$             | 2       |                  | 20         |
| 15      | do    | 175        | 1          | $(Bu-O-BO)_2$ *      | 3       |                  | 15         |
| 16      | do    | 175        | 1          | $C_6H_5B(OH)_3$      | 3       |                  | 12         |
| 17      | Wood  | 185        | 1          |                      |         |                  | 45         |
| 18      | do    | 185        | 1          | $B(OH)_3$            | 5       |                  | 10         |

\*Butyl metaborate.

between about 30 and 40, and wood rosin has a foaming index between about 40 and 50. We have regularly been successful in depressing the foaming index of these rosins by about half, and in certain instances have eliminated their latent foaming tendency substantially completely.

The method by which the boron compounds of the present invention effect their results is not known, and we do not wish to be limited to any particular theory. Our evidence is that the effect of the boron compounds is in part to convert the alcohols to volatile form causing them to escape during the treatment and in part to convert the alcohols to boron ester or boron complex form. The invention will be further described with reference to the examples. These examples illustrate specific embodiments of the invention and are not to be construed as limitations thereon.

#### Examples 1-18

The following illustrate the decrease in the foaming index effected by treating commercial gum and wood rosins with various oxidic compounds of boron according to the invention.

In each example, 100 gm. of the particular rosin was heated to the temperature shown in the table in a glass vessel provided with thermometer and stirrer. The boron compound was slowly added with vigorous stirring and the rosin was maintained at reaction temperature for an

hour thereafter. The foaming index of the rosin was then determined, and in certain instances the acid number as well.

#### Example 2

The following illustrates the manufacture of non-foaming fortified rosin size according to the present invention, and shows that the treatment with boron does not affect the utility of the rosin.

To gum rosin at 200° C. was slowly added 1% of boric acid with vigorous stirring. After 15 minutes 5% by weight of maleic anhydride was then added as fortifying agent. The maleic anhydride was allowed to react at 200° C. for two hours and the 70% solids, 12% free acid liquid rosin size which was tested for foaming, according to the method of Example 1.

The procedure was repeated except that the rosin was reacted with a maleic anhydride first and the boric acid thereafter. The results are as follows:

| Sequence of reaction:              | Foaming index |
|------------------------------------|---------------|
| Boric acid first, then maleic anh. | 7             |
| Maleic anh. first, then boric acid | 10            |

The results show that it is advantageous to postpone

admission of the fortifying agent until the boron compound has reacted.

We claim:

1. A method of treating a rosin having a latent foaming tendency because of the presence therein of organic alcohols, which comprises heating said rosin in molten form with an alcohol-reactive oxidic compound of boron at a temperature below the boiling point of said rosin and between 150° C. and 250° C.

2. A process according to claim 1 wherein the rosin is gum rosin.

3. A process according to claim 1 wherein the boron compound is boric acid.

4. A process according to claim 1 wherein the rosin is heated with sufficient of the boron compound and for a sufficient time to combine with between about one-third and three-quarters of said organic alcohols.

5. A process according to claim 1 wherein the temperature is between 175° C. and 200° C.

6. A method of manufacturing liquid rosin size from

15

5 a rosin having a latent foaming tendency because of the presence therein of organic alcohols, which comprises heating said rosin in molten form with an alcohol-reactive oxidic compound of boron at a temperature be-

tween about 150° C. and 250° C. and then saponifying the thus treated rosin with aqueous alkali metal alkali solution to form liquid rosin size.

7. A process according to claim 6 wherein the rosin, subsequent to heating with said boron compound and prior to said saponifying, is reacted with a fortifying agent.

8. A process according to claim 7 wherein the fortifying agent is maleic anhydride.

References Cited in the file of this patent

UNITED STATES PATENTS

|           |           |       |               |
|-----------|-----------|-------|---------------|
| 2,374,975 | Borglin   | ----- | May 1, 1945   |
| 2,448,621 | Rice      | ----- | Sept. 7, 1948 |
| 2,776,275 | Strazdins | ----- | Jan. 1, 1957  |